# EUROPEAN PATENT SPECIFICATION

(11) **EP 2 976 437 B1**
(45) Date of publication and mention of the grant of the patent: **15.05.2019**
(21) Application number: 14771156.8
(22) Date of filing: 19.03.2014
(51) Int. Cl.: C21D 1/20, C21D 8/00, C21D 7/13, C22C 38/00, C22C 38/02, C22C 38/04, C22C 38/12, C22C 38/14, C22C 38/22, C22C 38/24, C22C 38/28, C22C 38/32, C22C 38/34, C22C 38/38, C21D 6/00, C21D 1/09, C21D 1/18

(54) **AIR-HARDENABLE BAINITIC STEEL WITH ENHANCED MATERIAL CHARACTERISTICS**
LUFTHÄRTENDER BAINITISCHER STAHL MIT VERBESSERTEN MATERIALEIGENSCHAFTEN
ACIER BAINITIQUE DURCISSABLE À L'AIR AYANT DES CARACTÉRISTIQUES DE MATÉRIAU AMÉLIORÉES

(30) Priority: 22.03.2013 US 201313848829
(43) Date of publication of application: 27.01.2016
(73) Proprietor: Caterpillar, Inc., Peoria, IL 61629 (US)
(72) Inventor: LIU, Tianjun, Edwards, IL 61528 (US); KISER, Matthew Thomas, Chillicothe, IL 61523 (US)
(74) Representative: BRP Renaud & Partner mbB Rechtsanwälte Patentanwälte Steuerberater
(86) International application number: PCT/US2014/031201
(87) International publication number: WO 2014/153398

(56) References cited:
- EP-A1- 1 069 198
- JP-A- H08 176 733
- JP-A- 2012 237 040
- JP-A- 2013 028 840
- US-A- 5 601 667
- US-A- 5 660 648
- US-A1- 2007 119 519
- US-A1- 2007 227 634
- US-A1- 2012 288 397

## Description

### Technical Field

The present disclosure relates generally to an air-hardenable bainitic steel and, more particularly, to an air-hardenable bainitic steel with enhanced material characteristics.

### Background

Structural components for machinery, such as track links used on the undercarriage of track-type earth moving machines, are required to have material characteristics that include good yield strength, good wear resistance, good toughness, and good rolling contact fatigue resistance. Track links used on the tracks of a track-type machine such as a bulldozer or other earth moving equipment are well known in the industry. A track link typically has a lower portion, or the body of the link, and an upper portion, or the rail portion of the link. It is important that the rail portion of the track link have high surface hardness, whereas the body portion of the track link can have lower surface hardness for increased machinability. A high surface hardness in the rail portion is necessary because the rail portion is subjected to severe wear and spallation from continuous contact with track rollers. A lower surface hardness in the body portion of the track link allows holes for bushings to be more easily machined into the body portion. The lower surface hardness of the body portion of the track link also allows for a press fit between a bushing and the hole in the track link body without creating excessive residual stresses.

The manufacturing processes for obtaining the desired material characteristics in a track link or other structural component have typically included hot forging the component from a steel billet, followed by cooling, reheating to austenization temperatures, quenching, and tempering. These heat treatment processes may then be followed by additional heating of at least select portions of the component, quenching again, and tempering again before the final machining. Processing of a track link includes first heating a steel part to approximately 1150 - 1350 degrees C to bring the material to an austenite phase field, and then hot forging the part. The part is then slowly cooled to room temperature, followed by two heat treatment processes. In the first heat treatment process the track link is reheated to austenization temperature, quenched to room temperature, and then tempered to a hardness of approximately 30 - 39 Rockwell C hardness (HRC). In the second heat treatment process just the rail portion of the track link is locally reheated by induction, quenched to room temperature, and tempered to a hardness of 51 - 57 HRC. These heat treatment processes result in the track link having a hard rail and a softer body. The body of the link is then machined into final shape. The heat treatment processes add significantly to the expense of producing the components, and also require significant capital expenditures for furnaces, as well as ongoing maintenance expenses.

One attempt to produce alternative types of steel having good wear and rolling contact fatigue resistance coupled with improved levels of ductility toughness and weldability is described in U.S. Patent No. 5,879,474 to Bhadeshia ("the '474 patent") that issued on March 9, 1999. The '474 patent discloses a steel for use in making a steel rail, where the steel is purported to provide a high strength, wear and rolling contact fatigue resistant microstructure comprising carbide free "bainite" with some high carbon martensite and retained austenite in the head of the rail.

Although the alloy steel disclosed in the '474 patent may provide improved wear and rolling contact fatigue resistance, still further improvements in manufacturing costs and material characteristics may be possible. In particular, the '474 patent describes the use of significant quantities of expensive alloying elements such as Chromium (Cr) and Molybdenum (Mo) to achieve improved levels of rolling contact fatigue strength, ductility, bending fatigue life and fracture toughness, coupled with rolling contact wear resistance similar to or better than those of the current heat treated pearlitic rails.

EP 1 069 198 A1 relates to a machine structural steel product.

US 2007/227634 A1 relates to a forged or stamped average or small size mechanical part.

JP 2013-028840 A relates to a steel for induction hardening.

JP 2012-237040 A relates to a steel for spring parts.

The bainitic microalloyed steel produced in accordance with the chemistry and processes of the present disclosure solves one or more of the problems set forth above and/or other problems in the art.

### Summary

In one aspect, the present disclosure is directed to a method of producing a forged steel part according to claim 1.

In another aspect, the present disclosure is directed to a forged air-hardened bainitic steel part according to claim 4.

Further embodiments of the present invention are set out in the dependent claims.

### Brief Description of the Drawings

Fig. 1 is a schematic diagram of an exemplary disclosed process eliminating typical heat treating steps;
Fig. 2 is a continuous cooling transformation (CCT) diagram for producing the microstructure of an exemplary embodiment of the disclosure; and
Fig. 3 is a flowchart depicting an exemplary disclosed method that may be used to produce an exemplary microalloyed bainitic steel with enhanced characteristics.

### Detailed Description

A microalloyed, forged air-hardened, predominantly bainitic steel part with enhanced strength, wear, and toughness characteristics is disclosed. The microalloyed, bainitic steel may be economically produced without requiring many of the heat treatment processes previously thought necessary to achieve desired strength, wear, and toughness characteristics. As shown in Fig. 1, the typical heat treatment processes following hot forging of a steel part may include cooling, reheating to austenization temperature, quenching, and tempering. These heat treatment processes may then be followed by reheating select portions of the steel part a second time using induction, quenching a second time, and tempering a second time before the final machining. At least the first sequence of heat treatment steps involving reheating, quenching, and tempering may be required with conventional hot forging processes in order to obtain desired strength and toughness characteristics, while at the same time ending up with a part that is not too hard for machining. Significant cost savings may be achieved if at least some of these intermediate heat treatment processes can be eliminated. Capital investments for heat treatment capacity, and maintenance costs on the furnaces and other equipment may be reduced. In certain implementations of this disclosure the microalloyed, bainitic steel may be provided with the necessary composition and cooling after hot forging to arrive at a hardness of approximately 50 - 55 Rockwell C hardness (HRC) without even requiring the induction reheating, quenching, and tempering before final machining.

A predominantly bainitic microstructure according to various implementations of this disclosure is a microstructure that consists of at least 50% by volume of a bainitic microstructure. Certain embodiments may have at least 70% by volume of a bainitic microstructure. Other embodiments may have at least 85% by volume of a bainitic microstructure. Bainite is a microstructure that forms in steels at temperatures of approximately 250-550 °C (depending on alloy content). Bainite is one of the decomposition products that may form when austenite (the face centered cubic crystal structure of iron) is cooled past a critical temperature of 727 °C (1340 °F) depending on alloy content. A bainitic microstructure may be similar in appearance and hardness characteristics to tempered martensite.

A fine, non-lamellar structure, bainite commonly consists of cementite and dislocation-rich ferrite. The high concentration of dislocations in the ferrite present in bainite makes this ferrite harder than it normally would be. As shown in the continuous cooling transformation (CCT) diagram of Fig. 2, the temperature range for transformation to bainite (250-550 °C) is between those for pearlite and martensite. When formed during continuous cooling, the cooling rate to form bainite is more rapid than that required to form pearlite, but less rapid than that required to form martensite (in steels of the same composition). In accordance with various implementations of this disclosure, a microalloyed steel having the chemistry discussed in more detail below may be initially heated to austenization temperatures of approximately 1150 - 1350 °C or greater. The steel may then be hot forged into the desired shape, and control cooled from the forging temperature to achieve a bainitic microstructure. For the cooling after hot forging, atmospheric cooling or forced air cooling using a blower may be conducted. According to the present invention, the steel is cooled rapidly down to the eutectoid transformation temperature, and then cooled slowly over a range from 900 to 500 °C.

The cooling rate may be determined by reference to a CCT diagram, to know the range for cooling rates passing through the bainite transformation region and, thereby, controlling to the determined cooling rate range. The CCT diagram may have been previously prepared, stored in a database, or otherwise made available for control of the cooling process. The forged product is air cooled using fans or other means of circulating the cooling air to achieve a cooling rate that falls within the range from 0.5 to 5 °C per second, or 30 to 300 °C per minute, when cooling between approximately 900 °C and 500 °C. Most alloying elements will lower the temperature required for the maximum rate of formation of bainite, though carbon is the most effective in doing so. Bainite generally has a hardness that is greater than the typical hardness of pearlite and less than the hardness of martensite. Pearlite in the microstructure may contribute to reduced toughness. The composition and processing of the microalloyed steel according to various embodiments of this disclosure are selected to avoid or at least minimize the amount of pearlite present. In commercial practice a small amount of pearlite, such as less than 2 percent by volume, may unavoidably be present, particularly in the center of large sections, but care is taken to minimize its presence and effects.

The bainite microstructure essentially has a two-phase microstructure composed of ferrite and iron carbide or cementite. Depending on the composition of the austenite during the hot forging process, and the cooling rate after hot forging, there is a variation in the morphology of the resulting bainite. The resulting microstructures are referred to as upper bainite or lower bainite. Upper bainite can be described as aggregates of ferrite laths that usually are found in parallel groups to form plate-shaped regions. The carbide phase associated with upper bainite is precipitated at the interlath regions, and depending on the carbon content, these carbides can form nearly complete carbide films between the lath boundaries. Lower bainite also consists of an aggregate of ferrite and carbides. The carbides precipitate inside of the ferrite plates. The carbide precipitates are on a very fine scale and in general have the shape of rods or blades. For this reason, the bainitic microstructure becomes useful in that no additional heat treatments are required after initial cooling to achieve a hardness value between that of pearlitic and martensitic steels. The material characteristics of the microalloyed and forged steel can vary over a large range depending on the particular types and quantities of alloying elements included in the composition. When steel contains sufficient amounts of Si and/or Al, the carbide formation can be significantly retarded such that carbide does not have enough time to form during the continuous cooling process, resulting in a mixed microstructure of bainitic ferrite and retained austenite. This type of bainitic microstructure may be referred to as "carbide free" bainite. It has been found that such bainite may provide superior toughness to conventional types of bainite. The composition of alloying elements included in accordance with various embodiments of this disclosure results in a steel part having the strength, hardness, and toughness characteristics previously only achieved by including the intermediate heat treatment steps following hot forging of reheating to austenization temperature, quenching, and tempering.

The advantageous material characteristics discussed above are found to be achieved to a greater extent as the percentage by volume of bainitic microstructure is increased. Accordingly, a part that is 70% by volume bainitic microstructure may exhibit greater strength, hardness, and toughness characteristics than a part that is 50% by volume bainitic microstructure balanced with ferrite and/or pearlite type of microstructure. Additionally, a part that is 85% or greater by volume bainitic microstructure may exhibit even further enhanced characteristics of strength, hardness, and toughness than the part that is 70% by volume bainitic microstructure balanced with ferrite and/or pearlite type of microstructure. As shown in Fig. 1, intermediate heat treatment steps of reheating to austenization temperature, quenching, and tempering may be eliminated before the final machining of a forged product in accordance with various implementations of this disclosure. Induction reheating of select portions of the steel part, such as the rail portion of a track link used in contact with the tracks on earth moving machinery, may be included to achieve enhanced hardness and strength characteristics for certain parts or portions of parts. The increased hardness can also improve the wear resistance of the selected portions of the steel part. The alloying elements that are added to the composition in accordance with various embodiments of this disclosure may also be selected to obtain the desired volume percentages of bainitic microstructure throughout the part, regardless of the different cooling rates that may be experienced in different sections or portions of the part having different thicknesses.

It has been discovered in various implementations of this disclosure that the bainitic microstructure obtained after controlled air-cooling may also exhibit the same or similar hardness and strength characteristics as were previously achieved by following hot forging with quenching, reheating, quenching again, and tempering. A microalloyed steel may exhibit a martensitic microstructure after rapid cooling from hot forging temperatures through quenching in oil or water. The martensitic microstructure may have a Rockwell C hardness (HRC) of 50 after quenching depending on the carbon content of the steel. Typical methods of processing this martensitic microstructure steel may then include reheating back up to austenitic temperatures of approximately 800 °C - 950 °C, quenching again, and then tempering by reheating again to approximately 500 °C - 590 °C in order to soften the steel to approximately HRC 30. The controlled air cooling process for producing a predominantly bainitic microstructure according to various implementations of this disclosure may result in the same hardness of HRC 30 without all of the quenching, reheating, quenching and tempering steps previously required. As mentioned above, the predominantly bainitic microstructure may contain greater than 50% by volume of bainitic microstructure. The hardness after air cooling in accordance with this disclosure falls within the range from approximately 35 - 45 HRC.

The microalloyed steel according to various implementations of this disclosure has a chemical composition, by weight, as listed in Table 1:

**Table 1: Composition of microalloyed steel in weight percent.**

| Constituents | Concentration by weight (%) |
|---|---|
| Carbon | 0.25 - 0.35 |
| Manganese | 1.50 - 3.00 |
| Titanium | 0.02 - 0.06 |
| Vanadium | 0.00 - 0.10 |
| Silicon | 0.30 - 2.00 |
| Optional Nitrogen | 0.0050 - 0.0150 |
| Sulfur | 0.015 - 0.04 |
| Optional Chromium | 0.00 - 0.40 |
| Optional Molybdenum | 0.00 - 0.05 |
| Optional Boron | 0.00 - 0.003 |
| Iron and other residual elements | Balance |

Carbon (C) contributes to the attainable hardness level as well as the depth of hardening. In accordance with various implementations of this disclosure, the carbon content is at least 0.25 % by weight to maintain adequate core hardness after tempering and is no more than 0.35 % by weight to assure resistance to quench cracking and steel toughness. It has been found that if the carbon content is more than 0.35 % by weight, water quenching may cause cracking or distortion in complex-shaped articles and, in such cases, a less drastic quench medium such as oil may be required. Therefore, the range of C is from 0.25 - 0.35 wt.%. The microalloyed, bainitic steel according to various implementations of this disclosure may be air cooled in accordance with select cooling curves on the CCT diagram of Fig. 2.

Manganese (Mn) is a low cost material and contributes to the deep hardenability and is therefore present in most hardenable alloy steel grades. The disclosed alloy steel contains manganese in an amount of at least 1.50% by weight to assure adequate core hardness and contains no more than 3.00% to prevent manganese segregation and the formation of blocky retained austenite.

Silicon (Si) in amounts between approximately 0.30 - 2.00 wt.%, along with the Mn, allows the steel according to this disclosure to form a predominantly bainitic microstructure following air cooling from hot forging temperatures. The Si may also help deoxidation of the molten steel, as well as contributing to the formation of a carbide-free bainite with improved toughness when sufficient Si is added into the steel.

Chromium contributes to the hardenability of the present steel alloy and may be added in small amounts not exceeding 0.40 % by weight in order to allow for adjustment of the CCT curve to form a predominantly bainitic microstructure after air cooling. More Chromium increases steel cost.

Small amounts of other elements including Molybdenum (Mo) and Boron (B) may also be added to allow for further adjustment of the CCT curve to form a predominantly bainitic microstructure after air cooling.

Vanadium (V) and Nitrogen (N), despite their small quantities, may also be important ingredients in the present alloy steel composition, and may be added to provide precipitation hardening and to realize a consistently measurable enhancement of case and core hardness. Nitrogen combines with the titanium in the steel to form titanium carbonitrides to prevent grain coarsening during the reheat prior to forging and during the cooling after hot forging. Without Ti and N, the forged steel may have large prior austenite grain sizes, resulting in poor toughness.

The remainder of the alloy steel composition is essentially iron, except for nonessential or residual amounts of elements which may be present in small amounts. Titanium (Ti) is also provided in amounts between 0.02 - 0.06% to form titanium carbonitrides to prevent grain coarsening before and after forging. Sulphur (S), which in small amounts may be beneficial in that it promotes machining, is provided in amounts from 0.015 to 0.04 wt.% so as to not contribute to any loss of ductility and toughness. Phosphorus (P) in an amount over 0.05% may cause embrittlement, and preferably the upper limit should not exceed 0.035%. Other elements generally regarded as incidental impurities may be present within commercially recognized allowable amounts.

Manufactured articles, such as track links, having the above stated composition, may be advantageously initially formed to a desired shape by hot forging after heating up the microalloyed steel to austenization temperatures of approximately 1150 - 1350 °C. The formed articles are then controlled cooled as described above to produce a predominantly bainitic microstructure. Select portions of the hot forged articles, such as the rail portions of a track link, may then receive additional heat treatment by induction heating the select portions, quenching, and tempering before final machining to a desired final dimension.

Fig. 3 illustrates an exemplary method that may be used to produce a predominantly bainitic microalloyed steel part in accordance with various implementations of this disclosure. Fig. 3 will be discussed in more detail in the following section to further illustrate the disclosed concepts.

### Industrial Applicability

The steel and method of making the steel in accordance with various implementations of the present disclosure may reduce costs by eliminating heat treatment steps typically performed after hot forging. The disclosed microalloyed, forged, air-hardened bainitic steel may provide similar hardness, strength, and toughness characteristics to previously hot forged and heat treated steel parts, but without requiring all of the heat treatment processes. The microalloying elements in combination with the controlled air cooling may produce a predominantly bainitic microstructure after air cooling from hot forging temperatures. Select portions of the steel parts produced in accordance with the composition and processes of this disclosure may be further hardened if desired using localized induction heating followed by quenching and tempering.

The steel part produced in accordance with various advantageous implementations of this disclosure exhibits material characteristics that include a body hardness of 35 - 45 HRC after air cooling for good machinability with no heat treatment, a body yield strength that is greater than 1000 mega-pascals (MPa) after the air cooling, a hardness at the portions that have been additionally hardened through selective induction heating of greater than approximately 50 HRC, and a body toughness of approximately 20 Joules or greater in the Charpy impact test at room temperature.

As shown in Fig. 3, at step 320 a microalloyed steel having the composition shown above in Table 1 may be heated to austenization temperatures of 1150 degrees C to 1350 degrees C. The types of parts being manufactured in accordance with various implementations of this disclosure may include parts that require good machinability in at least one portion, high yield strength, good wear characteristics, and good toughness. One exemplary application of the disclosed compositions and processes is for track links used in the tracks of a track-type machine such as a bulldozer or other earth moving equipment. The size of the parts determines the size of a steel billet that is initially heated to austenization temperatures in accordance with step 320.

At step 322, the heated billet may be hot forged to a desired configuration. After the hot forging, step 324 may include air cooling the hot forged product at a cooling rate that results in the formation of a predominantly bainitic microstructure throughout the hot forged part. As shown by the CCT diagram of Fig. 2, the cooling rate may be chosen to avoid the formation of a large amount of martensitic microstructure or a predominantly ferrite and pearlite microstructure. In various implementations of this disclosure, the hot forged steel may be cooled at a rate that falls approximately in the range from 0.5 to 5 degrees C per second as the steel cools from 900 degrees C to 500 degrees C. In various alternative implementations, the weight percentages of the alloying elements in the composition of the steel may be varied in order to change the phase transformation curves on the CCT diagram, and achieve the desired predominantly bainitic microstructure at cooling rates achieved by transporting the hot forged steel parts along a conveyor at ambient temperatures. The microalloyed steel may also be advantageously provided with a composition that achieves the desired bainitic microstructure and hardness levels throughout the part even at the different cooling rates that may be experienced by different sections of the part having different thicknesses. The predominantly bainitic microstructure is a microstructure with greater than 50 % bainite, or advantageously greater than 70 % bainite, or more advantageously greater than 85 % bainite throughout the hot forged steel part. The hardness levels throughout the entire forged steel part after air cooling fall within the range from approximately 35 - 45 HRC.

At step 326, select portions of the steel part may be induction heated in order to achieve higher hardness levels. In the exemplary implementation of a track link, a high surface hardness may be desired for the rail portion because the rail portion may be subjected to severe wear from continuous contact with track rollers. A lower surface hardness in the body portion of the track link allows holes for bushings, pins, and bolts to be more easily machined into the body portion. The lower surface hardness of the body portion of the track link also allows for a press fit between a bushing and the hole in the track link body without creating excessive residual stresses. In various exemplary embodiments, the hardness of the induction heated portions of the steel part may fall within the range from approximately 50 - 57 HRC.

At step 328, after select portions of the steel part have been induction heated, at least these heated portions of the steel part may be quenched, using techniques such as directed sprays of quenching fluids onto the induction heated areas of the part. Following quenching, at step 330, the steel part may be reheated to tempering temperatures in order to improve its toughness. Final machining may then occur at step 332.

It will be apparent to those skilled in the art that various modifications and variations can be made to the disclosed microalloyed steel and method of forming the steel into a finished part without departing from the scope of the disclosure. Alternative implementations will be apparent to those skilled in the art from consideration of the specification and practice disclosed herein. It is intended that the specification and examples be considered as exemplary only, with a true scope of the disclosure being indicated by the following claims and their equivalents.

## Claims

1. A method of producing a forged steel part, comprising:
providing a steel billet having a composition consisting of, on a weight basis:
C: 0.25 - 0.35 wt.%,
Mn: 1.50 - 3.00 wt.%,
Si: 0.30 - 2.00 wt.%
V: 0.00 - 0.10 wt.%,
Ti: 0.02 - 0.06 wt.%,
S: 0.015 - 0.04 wt.%,
optional N: 0.0050 - 0.0150 wt.%,
Cr: 0.00 - 0.40 wt.%,
Mo: 0.00 - 0.05 wt.%,
B: 0.00 - 0.003 wt.%, and
a balance of Fe and incidental impurities;
heating the steel billet to an austenization temperature of 1150 degrees C to 1350 degrees C;
hot forging the steel billet to form the steel part; and
controlled air cooling the forged steel part after the hot forging,
wherein the controlled air cooling is carried out by rapidly cooling down the steel to the eutectoid transformation temperature and then cooling it slowly over a range from 900 to 500 °C at a cooling rate within the range from 0.5 to 5 °C per second.

2. The method according to claim 1, wherein the controlled air cooling is performed by moving the forged steel part along a conveyor at ambient temperatures.

3. The method according to claim 1, further including induction heating select portions of the forged steel part after the controlled air cooling, wherein the hardness of the select portions of the forged steel part after induction heating is greater than 50 HRC.

4. A forged air-hardened bainitic steel part obtainable by the method according to claim 1 and having a composition consisting of:
C: 0.25 - 0.35 wt.%,
Mn: 1.50 - 3.00 wt.%,
Si: 0.30 - 2.00 wt.%
V: 0.00 - 0.10 wt.%,
Ti: 0.02 - 0.06 wt.%,
S: 0.015 - 0.04 wt.%,
optional N: 0.0050 - 0.0150 wt.%,
Cr: 0.00 - 0.40 wt.%,
Mo: 0.00 - 0.05 wt.%,
B: 0.00 - 0.003 wt.%,
a balance of Fe and incidental impurities; and
a microstructure that is greater than 50% by volume bainitic microstructure throughout the entire steel part,
wherein the steel part has a body hardness of 35 - 45 Rockwell C hardness (HRC), a yield strength of greater than 1000 mega-pascals (MPa), and wherein the toughness of at least an inner portion of a body of the steel part is greater than or equal to 20 Joules at room temperature in accordance with the Charpy impact test.

## Patentansprüche

1. Verfahren zur Herstellung eines geschmiedeten Stahlteils, umfassend:
Bereitstellen eines Stahlwalzblocks mit einer Zusammensetzung, bestehend aus, auf Gewichtsbasis:
C: 0,25 - 0,35 Gew.-%,
Mn: 1,50 - 3,00 Gew.-%,
Si: 0,30 - 2,00 Gew.-%
V: 0,00 - 0,10 Gew.-%,
Ti: 0,02 - 0,06 Gew.-%,
S: 0,015 - 0,04 Gew.-%,
gegebenenfalls N: 0,0050 - 0,0150 Gew.-%,
Cr: 0,00 - 0,40 Gew.-%.
Mo: 0,00 - 0,05 Gew.-%,
B: 0,00 - 0,003 Gew.-% und
einem Rest von Fe und gelegentlichen Verunreinigungen;
Erwärmen des Stahlwalzblocks auf eine Austenisierungstemperatur von 1150°C bis 1350°C;
Warmschmieden des Stahlwalzblocks zum Bilden des Stahlteils; und
gesteuerte Luftkühlung des geschmiedeten Stahlteils nach dem Warmschmieden, wobei die gesteuerte Luftkühlung durchgeführt wird, indem der Stahl schnell auf die eutektische Transformationstemperatur abgekühlt und dann langsam über einen Bereich von 900 bis 500°C mit einer Abkühlrate im Bereich von 0,5 bis 5°C pro Sekunde abgekühlt wird.

2. Verfahren nach Anspruch 1, wobei die gesteuerte Luftkühlung durchgeführt wird, indem das geschmiedete Stahlteil entlang eines Förderbandes bei Umgebungstemperaturen bewegt wird.

3. Verfahren nach Anspruch 1, weiter beinhaltend das Induktionserwärmen von ausgewählten Abschnitten des geschmiedeten Stahlteils nach dem gesteuerten Luftkühlen, wobei die Härte der ausgewählten Abschnitte des geschmiedeten Stahlteils nach dem Induktionserwärmen größer als 50 HRC ist.

4. Geschmiedetes, luftgehärtetes bainitisches Stahlteil, das nach dem Verfahren nach Anspruch 1 erhältlich ist und eine Zusammensetzung aufweist, bestehend aus:
C: 0,25 - 0,35 Gew.-%,
Mn: 1,50 - 3,00 Gew.-%,
Si: 0,30 - 2,00 Gew.-%
V: 0,00 - 0,10 Gew.-%,
Ti: 0,02 - 0,06 Gew.-%,
S: 0,015 - 0,04 Gew.-%,
gegebenenfalls N: 0,0050 - 0,0150 Gew.-%,
Cr: 0,00 - 0,40 Gew.-%,
Mo: 0,00 - 0,05 Gew.-%,
B: 0,00 - 0,003 Gew.-%,
einem Rest von Fe und gelegentlichen Verunreinigungen; und
einer Mikrostruktur, die mehr als 50 Volumen - % bainitische Mikrostruktur über das gesamte Stahlteil aufweist,
wobei das Stahlteil eine Körperhärte von 35 - 45 Rockwell C - Härte (HRC), eine Streckgrenze von mehr als 1000 Megapascal (MPa) aufweist, und wobei die Zähigkeit von mindestens einem Innenabschnitt eines Körpers des Stahlteils größer oder gleich 20 Joule bei Raumtemperatur gemäß dem Charpy - Schlagversuch ist.

## Revendications

1. Procédé de production d'une pièce en acier forgé, comprenant :
se procurer une billette d'acier ayant une composition constituée par, sur une base en poids :
C : 0,25 à 0,35 % en poids,
Mn : 1,50 à 3,00 % en poids,
Si : 0,30 à 2,00 % en poids,
V : 0,00 à 0,10 % en poids,
Ti : 0,02 à 0,06 % en poids,
S : 0,015 à 0,04 % en poids,
N facultatif : 0,0050 à 0,0150 % en poids,
Cr : 0,00 à 0,40 % en poids,
Mo : 0,00 à 0,05 % en poids,
B : 0,00 à 0,003 % en poids, et
un complément de Fe et d'impuretés accidentelles ;
chauffer la billette d'acier jusqu'à une température d'austénisation de 1150 °C à 1350 °C ;
forger à chaud la billette d'acier pour former la pièce en acier ; et
refroidir sous air contrôlé la pièce en acier forgé après le forgeage à chaud,
dans lequel le refroidissement sous air contrôlé est effectué par refroidissement rapide de l'acier jusqu'à la température de transformation eutectoïde, puis refroidissement lent sur une plage allant de 900 à 500 °C à une vitesse de refroidissement se situant dans la plage allant de 0,5 à 5 °C par seconde.

2. Procédé selon la revendication 1, dans lequel le refroidissement sous air contrôlé est effectué par déplacement de la pièce en acier forgé sur un transporteur à des températures ambiantes.

3. Procédé selon la revendication 1, comportant en outre le chauffage par induction de parties choisies de la pièce en acier forgé après le refroidissement sous air contrôlé, la dureté des parties choisies de la pièce en acier forgé après le chauffage par induction étant supérieure à 50 HRC.

4. Pièce en acier bainitique durcie à l'air forgée pouvant être obtenue par le procédé selon la revendication 1 et ayant une composition constituée par :
C : 0,25 à 0,35 % en poids,
Mn : 1,50 à 3,00 % en poids,
Si : 0,30 à 2,00 % en poids,
V : 0,00 à 0,10 % en poids,
Ti : 0,02 à 0,06 % en poids,
S : 0,015 à 0,04 % en poids,
N facultatif : 0,0050 à 0,0150 % en poids,
Cr : 0,00 à 0,40 % en poids,
Mo : 0,00 à 0,05 % en poids,
B : 0,00 à 0,003 % en poids,
un complément de Fe et d'impuretés accidentelles ; et
une microstructure qui est supérieure à 50 % en volume de microstructure bainitique dans toute la pièce en acier,
la pièce en acier ayant une dureté de corps de 35 à 45 en dureté Rockwell C (HRC), une limite d'élasticité supérieure à 1000 mégapascals (MPa), et la ténacité d'au moins une partie interne d'un corps de la pièce en acier étant supérieure ou égale à 20 Joules à la température ambiante conformément à l'essai de résilience Charpy.
